

## UNITED STATES PATENT OFFICE

2,575,727

## METHOD OF COATING GLASSINE

Garrett H. Peters, Rhinelander, Wis., assignor to  
 Rhinelander Paper Company, Rhinelander,  
 Wis., a corporation of Wisconsin

No Drawing. Application November 12, 1947,  
 Serial No. 785,521

5 Claims. (Cl. 117—76)

1

The present invention relates to a method of coating paper, and more particularly, to a method of forming an adherent coating of a synthetic lacquer on glassine.

"Glassine" is a relatively transparent, grease-proof paper, formed of well hydrated cellulosic fibers, that has been super-calendered. Since glassine paper is inherently brittle, it is customary to plasticize glassine in order that it may be used satisfactorily in automatic wrapping machines. It has also been customary to coat glassine with wax in order to impart moisture-proofness and heat-sealing properties thereto. However, wax alone does not give entirely satisfactory heat-sealing properties.

It has therefore been proposed to employ thermoplastic resins for heat-sealing purposes. However, due to lack of adhesion between glassine and certain lacquers, for example thermoplastic resins, such as vinyl polymers and various rubber compositions, this proposal has not thus far gone into extensive commercial use. These lacquer films are too easily stripped from the glassine base to make satisfactory coated products.

The present invention provides a method whereby an adherent coating of synthetic lacquer may be applied to glassine or similar papers. The improved results of the method of the present invention are obtained by a pre-treatment of the glassine with an aqueous solution of a water-soluble, inorganic salt. Preferably, salts are employed which may be mixed with the plasticizers for joint application to the web on the paper machine. The aqueous solution of the salts and of the plasticizers may suitably be applied to the web by means of a size press located between sections of the driers. Thus, it is not necessary to provide a separate dampener or other means for applying the aqueous solution to the paper. Alternatively, prior to the super-calendering step, the machine finished grease-proof paper may be passed through a dampener containing an aqueous solution of the salt. The super-calendered and finished glassine is then passed through suitable coating apparatus, such as a conventional roller coating machine, by means of which the synthetic lacquer may be applied to the treated glassine.

I have found that the alkaline metal and ammonium salts, and particularly the sodium, potassium and ammonium salts, of polyvalent, slightly ionized inorganic acids are suitable for use in the process of the present invention. The alkali metal and ammonium salts of such polyprotic acids as carbonic acid, orthophosphoric acid, pyrophosphoric acid, metasilicic acid, orthosilicic acid and mixtures of silicic acids may be employed in the present invention. I have found that various synthetic resinous lacquers may be employed in the process of the present

2

invention, including vinyl resins, such as the copolymers of vinyl acetate and vinyl chloride, cyclized rubbers, and chlorinated rubbers.

The coated product obtained by the use of the present invention has enhanced transparency in comparison with glassine itself, and the added advantages of high moisture resistance, of ability to heat seal at relatively low temperatures, and of improved flexibility. These desirable characteristics are obtained along with a strong adherence of the coating film to the glassine base.

It is, therefore, an important object of the present invention to provide a method for coating glassine with a resinous lacquer composition to form an adherent film of the lacquer on the surface of the glassine.

It is a further important object of the present invention to provide a method of pre-treating glassine so that a resinous lacquer composition subsequently applied to the glassine surface will be strongly adherent thereto.

It is a still further object of the present invention to provide a method of coating glassine with a resinous lacquer which comprises pre-treating the glassine with an aqueous solution of an alkali metal or ammonium salt of a polyvalent and slightly ionized inorganic acid.

It is a yet further object of the present invention to provide a method for the preparation of coated glassine which comprises treating the surface of the glassine with an aqueous solution of a compound selected from the group consisting of alkali metal and ammonium carbonates, silicates and phosphates, and thereafter applying a synthetic thermoplastic lacquer composition to the treated surface of the glassine.

Other and further important objects of this invention will become apparent from the following description and appended claims.

As has been hereinbefore stated, the aqueous salt solution of the present invention comprises an aqueous solution of an alkali metal or ammonium salt of a polyvalent, slightly ionized inorganic acid. I have found that the alkali metal and ammonium salts of such polyprotic acids as carbonic acid, phosphoric acid, pyrophosphoric acid, metasilicic acid and orthosilicic acid are suitable salts for use in the present invention. I have found that the sodium and potassium carbonates, phosphates and silicates and ammonium secondary phosphate are particularly desirable salts for such use.

The concentration of the salt solution is dependent upon the solubility of the salt in water at the temperature employed. I have found that solutions which are of sufficient concentration to deposit from 1 to 5% of the salt based on the air-dry weight of the fiber in the paper are operative to give the improved results of the pres-

ent invention. Of course, more concentrated solutions may be employed, but since a larger amount is not necessary, it would not be commercially desirable to employ amounts in excess of about 5% by weight.

The thermoplastic resins which may be deposited on a treated glassine in accordance with the method of the present invention are preferably resinous lacquers which form a transparent, adherent film on the treated glassine surface. I have found various resinous lacquers, including copolymers of vinyl chloride and vinyl acetate, chlorinated rubbers, and cyclo-rubbers may be employed. These lacquers are suitable not only because of the excellent physical properties and chemical resistance of the compositions, but also for the heat-sealing properties of the lacquers.

As has been hereinbefore stated, the salt solution may be applied to the web on the paper machine in intimate mixture with the plasticizer employed in the preparation of the glassine, or, alternatively, the salt solution may be applied to the paper by a size press prior to the supercalendering operation. It is preferred that the aqueous salt solution be applied to the web in mixture with the plasticizers, since this method eliminates the necessity of a separate dampening bath or other apparatus for use in the application of the salt solution to the paper.

The resinous lacquer may be applied to the treated glassine by any suitable method. It is preferred that the application of the lacquer be carried out in a coating apparatus such as a conventional double-roller coating machine. By the use of such a double-roller coating machine, both sides of the glassine may be simultaneously coated with the resinous lacquer. Following the application of the resinous lacquer as a solution to the treated surfaces, the wet glassine is heated, as by passing the coated product through a drying tunnel, to evaporate the solvents from the lacquer and also to effect curing of the coated product.

Without limiting my invention to any particular procedure, the following example, in which parts by weight are given, will serve to illustrate my method in its preferred form.

#### EXAMPLE

Glassine was coated in accordance with the present invention as follows:

The paper was made from wood pulp on a Fourdrinier paper making machine. The web on the machine was passed through a tank containing plasticizer and an aqueous solution of a

suitable salt as hereinbefore described. The treated paper is then super-calendered by conventional methods used in the manufacture of glassine. The glassine thus prepared was then

5 passed through the rollers of a double-roller coating machine having horizontal parallel rolls placed one above the other. The bottom roll ran in a pan of lacquer and coated the lower surface of the glassine. The upper surface of the glassine is coated by lacquer pumped from the lower lacquer pan and sprayed on the upper surface ahead of the upper roll. Any excess lacquer was removed from the coated glassine by the squeezing action of the rolls. The wet coated glassine is then passed to a drying tunnel maintained at a temperature of 150° to 200° F. to evaporate solvent from the lacquer.

The results obtained from the use of a representative group of salts, selected from the alkali

20 metal and ammonium phosphates, carbonates and silicates, in combination with two types of suitable resinous lacquers are tabulated in the following tables. The physical properties of the coated glassines were determined on coated products

25 obtained by the use of a salt concentration which was sufficient to deposit 1, 2, and 5% of salt based on the weight of fiber in the paper. Each of the three concentrations has been found satisfactory, however, for clarity and brevity only those results obtained at a concentration of 5% are presented.

The resinous lacquer compositions employed are as follows:

#### Number I

| Parts by Weight | Component                                                                                                                          |
|-----------------|------------------------------------------------------------------------------------------------------------------------------------|
| 61.6            | Copolymer of vinyl acetate and vinyl chloride.                                                                                     |
| 26.4            | Copolymer of vinyl acetate, vinyl chloride, and maleic anhydride.                                                                  |
| 12.0            | Plasticizer for copolymer (butyl phthalyl butyl glycolate, $\text{C}_6\text{H}_5\text{OCOC}_6\text{H}_4\text{COOC}_6\text{H}_5$ ). |
| 20.0            | Paraffin wax (M. P. 133-135° F.).                                                                                                  |
| 135.0           | Methyl ethyl ketone.                                                                                                               |
| 225.0           | Toluene.                                                                                                                           |

#### Number II

| Parts by Weight | Component                         |
|-----------------|-----------------------------------|
| 92.0            | Cyclorubber.                      |
| 8.0             | Paraffin wax (M. P. 133-140° F.). |
| 400.0           | Toluene.                          |

In the following tables the following symbols have the indicated significance: Ex—excellent, G—good, F—fair.

| No.  | Salt                              | Per Cent by Wt. of Salt Retained | pH (Salt Sol) | Lacquer | Adhesion | Transparency | Color | Gloss |
|------|-----------------------------------|----------------------------------|---------------|---------|----------|--------------|-------|-------|
| 1... | $\text{Na}_4\text{P}_2\text{O}_7$ | 5                                | 8.60          | I       | Ex       | 67           | F     | F     |
| 2... | $\text{Na}_3\text{PO}_4$          | 5                                | 7.31          | I       | Ex       | 72           | F     | F     |
| 3... | $\text{Na}_2\text{HPO}_4$         | 5                                | 6.80          | I       | Ex       | 76           | G     | G     |
| 4... | $\text{NaH}_2\text{PO}_4$         | 5                                | 4.46          | II      | Ex       | 73           | Ex    | G     |
| 5... | $(\text{NH}_4)_2\text{HPO}_4$     | 5                                | 6.21          | I       | G        | 74           | F     | F     |
| 6... | $\text{NaHCO}_3$                  | 5                                | 9.15          | I       | Ex       | 84           | F     | Ex    |
| 7... | $\text{Na}_2\text{CO}_3$          | 5                                | 9.27          | I       | Ex       | 59           | F     | F     |
| 8... | $\text{Na}_2\text{SiO}_3$         | 5                                | 8.61          | I       | Ex       | 53           | F     | F     |
| 9... | $\text{Na}_2\text{SiO}_3$         | 5                                | 8.44          | I       | Ex       | 70           | F     | G     |

It will, of course, be understood that various details of the process may be varied through a wide range without departing from the principles of this invention, and it is, therefore, not the purpose to limit the patent granted hereon otherwise than necessitated by the scope of the appended claims.

I claim as my invention:

1. A method of coating glassine which comprises treating glassine stock in web form with an aqueous solution consisting essentially of a salt selected from the group consisting of alkali metal and ammonium phosphates, silicates and carbonates, drying the thus treated glassine stock and applying to said treated surface a resinous lacquer in which the resinous constituent consists of a thermoplastic resin selected from the group consisting of cyclized rubbers, chlorinated rubbers, and a vinyl co-polymer consisting of vinyl chloride and vinyl acetate, which resinous constituents do not adhere well to glassine when not so treated.

2. In a method of coating glassine with a resinous lacquer composition containing paraffin wax and in which the resinous constituent consists of a thermoplastic resin selected from the group consisting of cyclized rubbers, chlorinated rubbers, and a vinyl copolymer consisting of vinyl chloride and vinyl acetate, which lacquer compositions do not adhere well to glassine, the improvement which comprises treating the glassine stock in web form with an aqueous solution consisting essentially of a salt selected from the group consisting of alkali metal and ammonium phosphates, silicates and carbonates, and supercalendering and drying the thus treated glassine stock prior to the application to said treated glassine stock of said resinous lacquer composition, whereby the adhesion of said resinous lacquer composition to said surface is improved.

3. In a method of making a coated glassine including the steps of supercalendering a dampened web of well hydrated cellulosic fibers, the improvement which comprises treating said well hydrated cellulose fibers in web form with an aqueous dampening solution of a salt selected from the group consisting of alkali metal and ammonium phosphates, carbonates and silicates, supercalendering the thus treated web to thereby dry and finish the same and applying thereto a resinous lacquer in which the resinous constituent consists of a thermoplastic resin selected from the group consisting of cyclized rubbers, chlori-

nated rubbers, and a vinyl co-polymer consisting of vinyl chloride and vinyl acetate, which resinous constituents normally do not adhere well to untreated glassine, whereby the adherence of the resinous constituent so selected is improved.

4. In a method of coating glassine with a resinous lacquer composition in which the resinous constituent consists of a vinyl co-polymer consisting of vinyl chloride and vinyl acetate that does not adhere well to an untreated glassine, the improvement which comprises treating glassine stock in web form with an aqueous solution consisting essentially of a salt selected from the group consisting of alkali metal and ammonium phosphates, silicates and carbonates, drying the thus treated glassine stock and thereafter applying to said treated surface said vinyl co-polymer, the treatment with said aqueous solution serving to improve the adherence of said vinyl co-polymer to the glassine stock.

5. In a method of coating glassine with a vinyl co-polymer consisting of vinyl chloride and vinyl acetate, which co-polymer normally does not adhere well to glassine, the improvement which comprises first treating glassine stock in web form with an aqueous solution consisting essentially of a salt selected from the group consisting of alkali metal and ammonium phosphates, silicates and carbonates, drying the thus treated glassine stock and subsequently applying to said treated surface said vinyl co-polymer consisting of vinyl chloride and vinyl acetate as aforesaid, the treatment of said glassine with said aqueous salt solution serving to improve the adherence of said co-polymer to said glassine stock.

GARRETT H. PETERS.

#### REFERENCES CITED

40 The following references are of record in the file of this patent:

#### UNITED STATES PATENTS

| Number    | Name                | Date          |
|-----------|---------------------|---------------|
| 524,024   | Howe -----          | Aug. 7, 1894  |
| 1,597,840 | Summers -----       | Aug. 31, 1926 |
| 2,058,961 | Dozier -----        | Oct. 27, 1936 |
| 2,163,085 | Cupery -----        | June 20, 1939 |
| 2,244,795 | Williams -----      | June 10, 1941 |
| 2,268,674 | Roth -----          | Jan. 6, 1942  |
| 2,291,616 | Fletcher -----      | Aug. 4, 1942  |
| 2,300,373 | Stoner et al. ----- | Oct. 27, 1942 |
| 2,333,023 | Manor -----         | Oct. 26, 1943 |
| 2,403,697 | Wenberg -----       | July 9, 1946  |